

# United States Patent

Mowat

[15] 3,645,736

[45] Feb. 29, 1972

[54] **PHYSICAL DEVELOPMENT SYSTEMS,  
PROCESSES AND RELATED  
MATERIALS**

[72] Inventor: Lois E. Mowat, Waltham, Mass.

[73] Assignee: Itek Corporation, Lexington, Mass.

[22] Filed: July 11, 1968

[21] Appl. No.: 743,983

[52] U.S. Cl..... 96/48, 96/60

[51] Int. Cl..... G03c 5/54

[58] Field of Search..... 260/430, 429 J; 96/48, 90,  
96/60

[56] **References Cited**

UNITED STATES PATENTS

3,152,903 10/1964 Shepard et al. .... 96/60

3,256,092 6/1966 Means et al..... 96/60  
3,458,316 7/1969 Viro..... 96/94

*Primary Examiner*—Norman G. Torchin

*Assistant Examiner*—John L. Goodrow

*Attorney*—Homer O. Blair, Robert L. Nathans and W. Gary  
Goodson

[57] **ABSTRACT**

This disclosure relates to a new and useful complex of silver ion with nitrilotriacetate ions which is particularly useful in sensitizing a photographic latent image on a photosensitive medium especially those in which the photosensitive component is a photoconductor. The complex can be applied to the photoexposed medium or formed on the medium before or during photoprocessing. Also described are methods of photoprocessing latent photographic images, especially by amplifying latent silver images with nonsilver metals such as copper and tin.

8 Claims, No Drawings

## PHYSICAL DEVELOPMENT SYSTEMS, PROCESSES AND RELATED MATERIALS

### BACKGROUND OF THE INVENTION

#### 1. Field of the Invention

This invention relates to a photographic physical developer and systems including the new developer.

#### 2. Description of the Prior Art

Physical development is a photographic development process distinguished from chemical development by the fact that metal required for contrast formation is largely supplied from the developer system whereas, in "chemical development," the contrast metal is present as metal ions in the crystal lattice of the grains on the film. Physical development is primarily used for development of latent images formed by light-activation of the photosensitive component of a photographic medium. In general, the physical development can be accomplished by contacting the latent image with the physical developer, e.g., a solution of reducible metal ion such as silver, mercury, gold, platinum or copper ions and a solution of a reducing agent for the selected metal ion, or, if desired, a latent metal image can be first formed by contacting the latent image with a solution of sensitizing ions, e.g., silver, followed by treatment with additional metal ions and a reducing agent therefor. The additional metal ions need not be the same as the sensitizing metal ions and when they differ the development is known as amplification since the metal latent image, i.e., germ metal image, is amplified, i.e., intensified, with the second metal. This latter process is of particular importance when the second metal is other than silver, a costly component of physical developer systems, but nevertheless an especially effective component, particularly in forming the latent metal image. Although many metals can be used for formation of the latent metal image in physical development, e.g., copper, gold, platinum, mercury, copper and the like, silver is at present the preferred metal. Particularly effective amplifying metals are silver, copper and tin, the latter two being preferred since they are more economical than silver but comparable in their action and effect.

Various literature articles and patents are available for description of the variety and types of photographic media with which physical development is employed to produce visible images corresponding to latent photographic images on the media. For example, U.S. Pat. Nos. 2,057,016; 2,750,292; 2,735,773; 2,183,447; and 3,072,542 describe the use of various physical developer systems used for image formation with various photosensitive media.

British Specification 1,043,250, describes physical developer systems for developing latent images on photosensitive media comprising a photoconductor, especially metal containing photoconductors, which are rendered chemically reducing when exposed to activating radiation, especially titanium dioxide.

One of the basic problems encountered in using physical developers is the efficiency of germ metal image site formation. The activation of the photosensitive component of the photographic media results in production of a number of sites of activation but, up to now, the conversion of these activation sites to a corresponding number of germ metal sites has fallen to considerably less than 100 percent efficiency for reasons which do not lend themselves to simple explanation. Thus, when physical developers are used, the initial photographic media appear to have a very low photographic speed whereas they can have high photographic speed but, due to the low efficiency of physical development, such high photographic speed is not apparent.

### SUMMARY OF THE INVENTION

It has now been unexpectedly found that improved physical development can be realized when the sensitizing metal ion is a complex of silver ion and an aminotrialkanoate ions, especially nitrilotriacetate ions, a new silver ion complex. In addition to the improvements realized with the new silver com-

plex, it has also been surprisingly found that silver ion, in the form of the complex, can be employed at concentrations considerably lower than concentrations normal to silver ion sensitizing of the prior art.

5 The silver ion complex, or either component thereof, can be applied to the photographic medium as such before or after photoexposure, or can be formed in situ by contacting the medium with a source of silver ions and a source of nitrilotriacetate ions, in whatever order. The source of nitrilotriacetate ions can be the developer of the amplifying solution. There is no limitation to the manner of application of the complex, whether as the complex or formed in situ on the latent image, except that the complex be available when the visible image formation takes place. In general, the improvements described hereinafter are realized by converting the photographic latent image to a latent silver image by contacting with silver ions in the presence of nitrilotriacetate ions. The resulting latent silver image can be amplified by any of the 10 art-recognized procedures by use of physical development procedures, to obtain visible images corresponding to the original photographic latent image.

Particularly effective in the important step of forming the 15 latent silver image is a solution of the new silver complex of this invention which merely need be contacted with the photographic latent image to obtain the latent silver image. Also useful are photographic media which contain a source of nitrilotriacetate ions with, or without, a source of silver ions which after photoexposure, will form the desired latent silver 20 image when the silver complex is activated as described hereinafter.

A particularly effective method of amplification of the 25 latent silver image involves the use of copper or tin amplification processes described in commonly assigned copending U.S. application Ser. Nos. 743,981 filed July 11, 1968 and 743,982 filed July 11, 1968, respectively.

### DESCRIPTION OF THE PREFERRED EMBODIMENTS

40 The present invention is particularly effective with photographic media the photosensitive component of which comprises a photoconductor which includes both organic and inorganic compounds and mixture of compounds. Preferred photoconductors are inorganic compounds such as compounds of a metal and a nonmetallic element of Group VIA of the Periodic Table\*, (\*Periodic Table from Lange's HANDBOOK OF CHEMISTRY, 9th Edition, pp. 56-57, 1956.) for example, metal oxides, such as zinc oxide, titanium dioxide, 45 antimony trioxide, aluminum oxide, zirconium dioxide, germanium dioxide, indium, stannic oxide, barium titanate, lead oxide, tantalum oxide, and tellurium oxide; metal sulfides such as cadmium sulfide, zinc sulfide and stannic sulfide; and metal selenides, such as cadmium selenide. Metal oxides are 50 generally preferred, and, of these titanium dioxide, because of the unusually good results obtained therewith.

A simple test useful in determining whether a selected 55 material has a photoconductor effect involves mixing the test material with an aqueous solution of silver nitrate. Little, if any, reaction should take place in the absence of light. On subjecting the test mixture to light such as ultraviolet light along with a control solution of silver nitrate, the rate of darkening of the test solution compared to the control solution is determined; if faster than the control solution, the test material is a photoconductor.

The photographic media comprise the photoconductor or an inert carrier sheet which comprise any suitable backing of sufficient strength and durability to satisfactorily serve as a reproduction carrier. The carrier sheet may be in any form 70 such as, for example, sheets, ribbons, rolls, etc. The sheet can be made of any suitable material such as wood, rag content paper, pulp paper, plastics, e.g., polyethylene terephthalate and cellulose acetate, cloth, metallic foil such as aluminum foil, and glass. The preferred form of the carrier sheet is a thin sheet which is durable and flexible.

The photoconductor is normally applied to the carrier with a binding agent. In general, these binders are translucent or transparent so that they do not interfere with transmission of light therethrough. Preferred binder materials are organic materials such as resins, e.g., butadienestyrene copolymers, poly (alkylacrylates) such as poly(methyl methacrylate), polyamides, polyvinyl acetate, polyvinyl alcohol and polyvinylpyrrolidones.

Other photographic media containing other photosensitive components than the aforementioned which are developed with physical developers are useful in this invention, for example, systems in which the photosensitive component is a diazonium salt or a diazosulfonate as described in the U.S. Pat. Nos. 2,183,447 and 2,750,292, respectively.

The exposure of the photographic medium can be by any of the art-recognized procedures such as described in the U.S. Patents and British Specification mentioned herein.

The new silver complex of the present invention is preferably formed in solution from a source of silver ions and a source of nitrilotriacetate ions. Suitable sources of the respective ions are readily known in the art and the selection of any particular source is a matter of choice and generally one of convenience. The most preferred source of silver ion is silver nitrate because it is readily available and constitutes the most common form. In addition, the solubility properties of silver nitrate make it eminently suited for the preparation of solutions of a wide range of concentrations. Other sources of silver ion can be used, even silver ion complexes which are not as stable as that of the present invention but no appreciable advantage is realized, for which reason, the nitrate salt is usually preferred. The complexing ion, nitrilotriacetate ion, can be formed in solution by dissolving any suitable source of the ion. Since the free acid itself is not appreciably dissociated in solution, it does not constitute a suitable source of the required ion. Preferably, a soluble salt of nitrilotriacetic acid is used as a source of the ion. Because of their high solubility in water and aqueous solvent systems, the preferred salts are ammonium and alkali metal salts (Na, K, Li), especially the sodium salts which are commercially available. Since the complexing ion is from a tribasic acid, it is possible to use each of the carboxyl groups for salt formation. Thus, it is possible to use, for example, the disodium as well as the trisodium salt. The reason for preference of the ammonium or alkali metal salts is the well known solubility of the most such salts regardless of the negative ions present in solution, e.g., the negative ions of the silver ion source. In photographic processing, the preference for systems in which various components have good water solubility is well-known to those skilled in the art and need not be fully explored for the purpose of this disclosure. Thus, the selection of sources of silver ions and nitrilotriacetate ions should be based at least in part on the possibility of precipitate formation between for example the negative ion of the source of silver ion and the positive ion of the source of nitrilotriacetate ions. However, even should the combination of ions from the respective sources, or from any source, including the solvent system, result in precipitate formation, this can be remedied by the mere expedient of separating the precipitate from the liquid phase, e.g., by filtration or centrifugation and decantation. Of course, the sources of the respective ions should be photographically acceptable, i.e., they should not adversely affect the photographic processing especially by establishing reactions competitive with the desired oxidation-reduction reactions characteristic of photographic processing.

As an alternative to forming the silver nitrilotriacetate complex in solution for use in the herein-described process, it is possible but needlessly tedious, to obtain a complex salt thereof, for example, by forming a supersaturated solution thereof, precipitating the complex salt and separating the precipitate. No appreciable advantage is obtained by this procedure and because it entails considerable difficulty it is generally avoided since the complex formed in solution is useful as such. Additionally, if the complex salt were obtained by

the aforementioned procedure, it would of necessity be dissolved in solution for use in the described photographic processing.

When used in the form of a sensitizing solution for application directly to the photographic latent image, results show that the concentration of the silver complex of this invention does not appear to be critical. For example, solutions containing as little as  $10^{-5}$  moles per liter have been used to sensitize latent images which on amplification gave excellent visible prints corresponding to the original latent image. Concentrations ranging up to saturation concentration can be used, but the preferred solutions are usually those of minimum concentration which will yield an effective latent silver image, for example from about  $1 \times 10^{-5}$  to about  $2 \times 10^{-1}$  moles per liter, although concentrations as low as  $1 \times 10^{-6}$  moles per liter are also operable. It is usually preferable to avoid higher concentrations if the source of nitrilotriacetate is an alkali metal salt due to the possible formation of silver oxide precipitate at extremely high pH values which result from such alkali metal salts. When the higher concentrations are desired, it is preferred to use ammonium salts or salts of weakly basic amines. The concentrations of the respective ions of the present new complex in solution need not be equimolar nor are they restricted to any specific stoichiometry since they may be varied appreciably in solution without adverse effect. As is obvious, too, the stoichiometry of the complex can also vary since the negative ion is trivalent and silver ion is monovalent. Most likely of the formulas of the complex ion is that in which one silver ion is combined with one nitrilotriacetate ion, with the complex having a residual charge of -2, especially when the sources of the respective ions are used as equimolar concentration. There is no absolute requirement for such equimolar concentration but it is usually preferred since best results are obtained therewith.

In lieu of using a solution of the present new silver complex, it is possible to form the complex in situ by, for example, incorporating the respective sources of the ions in the photographic medium prior to photoexposure, or alternatively, the source of nitrilotriacetate can be incorporated in the photographic medium prior to photoexposure and the medium contacted with silver ions after photoexposure. A further embodiment involves application of the nitrilotriacetate ion source in the developer of the subsequent physical development processing. When reference is made in this disclosure and in the appended claims to converting a photographic latent image to a latent silver image by contacting the latent image with silver ions in the presence of nitrilotriacetate ions, all of the foregoing embodiments are intended thereby.

Of these embodiments, the preferred is the photographic medium, especially that comprising a photoconductor, containing the source of nitrilotriacetate ions, with or without a source of silver ions. The said sources of ions can be applied together to form the complex on the photographic medium, or the respective sources can be maintained separately on the photographic medium, e.g., in microencapsulated form or in separate layers on the medium. When in separated form the photographic media are activated after photoexposure by pressuring the microencapsulated form or by merely exposing the medium to a solvent system which permits reactive contact of the respective ions to form the new silver complex. On activation, the complex then forms the latent metal image which is then subjected to further processing to produce a visible image. When the medium contains a source of only one of the ions of the new silver complex, the medium is activated after photoexposure by contacting with a solution of the other ion to form the desired complex.

If desired, the photographic media can contain other materials such as the developer and/or metal ions for the physical development processing steps which follow latent silver image formation. For example, the medium can contain any of the aforementioned amplifying metals, e.g., silver ions, copper ions, or stannous ions, or the reducing agents therefor. If desired, these additional materials can be present in

separate layers or microencapsulated form, which can be activated as described for the formation of the new silver complex of this invention.

In the foregoing description relative to inclusion of the new silver complex components and the said other materials, the preferred media are those comprising a photoconductor as the photosensitive component, preferably titanium dioxide.

After the formation of the latent silver image, the medium is then subjected to treatment with any of a variety of physical developer systems to obtain a visible image. The physical developers include the following:

A. Silver physical developer:

1. Silver ion, e.g., silver nitrate;
2. Reducing agent for silver ion, e.g., N-(p-hydroxyphenyl) glycine; N-methylaminophenol; ethylenediamines; hydroquinone; methylhydroquinone; ferrous compounds such as ferrous ethylenediaminetetraacetic acid and the like;
3. fixer for silver ion, e.g., thiosulfate or thiocyanate salts.

B. Copper physical developer:

1. Copper ions, e.g., cupric or cuprous ion
2. a reducing agent for copper ions, such as ascorbic acid, titanous and vanadous ion, and complexes of ferrous, titanous or vanadous ion with basic nitrogen-containing organic polycarboxylic acids, e.g., nitrilotriacetic acid, ethylenediaminetetraacetic acid and similar such acids.

C. Stannous physical developer:

1. stannous ions
2. a reducing agent fro stannous ions, e.g., chromous ions.

The additional silver ions of the silver physical developer may already be present on the medium from the sensitizing step with the new silver complex of this invention. In most cases it is preferred to add additional silver ion in the physical developing process but this is not always necessary.

If desired, prior to physical development, the latent silver image can be contacted with a reducing agent for silver which results in some amplification thereof with silver, the excess silver ion of the sensitizing solution being the source of reduced silver. The latent silver image can thus become at least partially visible.

When the amplifying metal is other than silver, it is preferable to remove substantially all traces of silver ion from the medium prior to physical development. When the initial sensitizing bath of the present new complex is of a low order concentration, e.g., less than  $10^{-3}$  molar, such removal is not always necessary. The removal can be by standard procedures, such as water-washing or complex formation, e.g., with thiosulfate ion.

Conveniently, thiosulfate ion can be included in the amplifying metal ion solution or in the reducing agent solution, thus obviating the need for a separate treatment step.

When the copper physical developer is used, it is preferred to use a solution of cupric ethylenediaminetetraacetic acid or cupric nitrilotriacetic acid as the copper source and a solution of titanous ethylenediaminetetraacetic acid or titanous nitrilotriacetic acid.

A further improvement in the overall processing to a visible amplified image is realized when a source of nitrilotriacetate ions is included in the solution of the reducing agent of the silver physical developer.

The principal improvements realized in the use of present new silver complex is an overall improvement in the apparent photographic speed of the photographic media treated therewith. The reason for the improvement is not necessarily fully understood, but seems to derive from a more efficient utilization of the original radiation activated sites of the medium in the formation of the silver latent image which is discussed hereinbefore. The applicant does not wish to be bound by the theoretical explanation, but it seems quite logical for the purpose of explaining the observed effects, as illustrated herein.

Additional advantage of the present new silver complex is the fact that it functions at extremely low silver concentrations where, in the absence of nitrilotriacetate ions, no detectable latent image is formed, or at best the latent image and the subsequently intensified image are weak, i.e., low density. The use of low concentrations of silver ion gives an obvious economic advantage, and, even further, also gives excellent results with a substantial reduction in the fog level of the developed photographic medium.

These desirable effects are apparently peculiar to the present new complex and are not shared by analogous complexes. For example, when nitrilotriacetate ion if replaced by ethylenediaminetetraacetate ions, the resulting complex is found to be even less effective than simple silver ion in solution in formation of the silver latent image; in many instances, no appreciable reduction of silver occurs from this complex on exposure to the photographic latent image, as evidenced by the lack of a visible image on physical development, or at best production of only a faint image.

In addition to its use in formation of silver latent images, the present new complex can also be used as a source of silver in electroplating baths and electroless plating baths, as a bacteriostat and for medical purposes for which silver nitrate is commonly used. In these uses, the complex is employed in the form of a solution, generally an aqueous solution.

#### EXAMPLE 1

30 A sheet of paper coated with titanium dioxide (as described in British Specification 1,043,250) is exposed for  $10^{-3}$  seconds on a sensitometer. After a 10 second wait, the sheet is immersed for 10 seconds in a solution which is 0.005 M silver nitrate and 0.005 M trisodium nitrilotriacetate and drained for 5 seconds. The paper is next immersed for 10 seconds in 200 ml. of a solution which is 0.48 M CuEDTA and 0.02 M sodium sulfite, mixed with 100 ml. of a solution containing 2.0 g./l. p-methylaminophenol and 7.5 g./l.  $\text{Na}_2\text{SO}_3$  and drained for 5 seconds. The paper in next immersed for 15 seconds in a solution of TiEDTA which is  $2.5 \times 10^{-3}$  M thiourea (TiEDTA developer) and drained for 5 seconds to obtain a visible image of good density and contrast.

45 The TiEDTA solution is prepared by adding 10 ml. of 20 percent titanous chloride solution to a solution of 25 ml. of 1 M Na<sub>2</sub>EDTA in 75 ml. of water.

Examination of stepwedges so prepared gives the following results.

| Sample | Nos. of steps | Optical Density |         |         |      |
|--------|---------------|-----------------|---------|---------|------|
|        |               | step 21         | step 20 | step 11 | Fog. |
| A      | 21+           | 1.30            | 1.30    | 1.03    | 0.18 |
| B      | 21+           | 1.30            | 1.28    | 1.02    | 0.18 |
| C      | 21+           | 1.28            | 1.25    | 0.95    | 0.15 |

55 For comparison, stepwedges prepared in the same manner but without nitrilotriacetate ions in the silver ion solution using show an average of 18 steps, and a somewhat lower density.

#### EXAMPLE 2

A paper coated with titanium dioxide is subjected to the following stepwise treatment:

- a. expose on sensitometer for  $10^{-3}$  seconds and hold for 10 seconds.
- b. immerse in 0.0025 M  $\text{AgNO}_3$  for 10 seconds and drain for 10 seconds.
- c. develop in 100 ml. of a solution of p-methylaminophenol (2g./l.) and  $\text{Na}_2\text{SO}_3$  (7.5 g./l.) to which is added 2.5 ml. 1 M  $\text{Na}_2\text{NTA}$  and drain for 10 seconds. The sheet is fixed by immersion for one minute in a solution (aqueous) of  $\text{Na}_2\text{S}_2\text{O}_4$ . A good black and white print is obtained; the stepwedge shows 19 steps.

## EXAMPLE 3

The procedure of Example 2 is repeated but the  $\text{Na}_3\text{NTA}$  at a 0.003 M concentration is present in the silver nitrate solution. The results show an increase of 2 steps over the print of Example 2, the total number of steps being 21.

## EXAMPLE 4

A paper sheet coated with titanium dioxide is exposed for  $10^{-4}$  seconds on a sensitometer and then treated by the procedure of Example 3 to obtain a dark gray image with 7 steps (stepwedge).

When this procedure is repeated using  $\text{Na}_3\text{NTA}$  (2.5 ml. of 1 M solution/100 ml.) in the developer solution, the number of steps increases to 9. When the silver ion concentration in the sensitizer solution is adjusted to 0.005 M, the number of steps increases to 11.

## EXAMPLE 5

Titanium dioxide-coated sheets are exposed for  $10^{-3}$  seconds held for 10 seconds and processed according to the following procedures:

## Procedure A

1. Immerse for 10 seconds in a solution of:

|                            |         |
|----------------------------|---------|
| $\text{AgNO}_3$ (0.005M)   | 100 ml. |
| 1M $\text{Na}_3\text{NTA}$ | 5 ml.   |

and drain for 10 seconds.

2. Immerse for 30 seconds in the CuEDTA solution containing silver developer described in Example 1.

## Procedure B

Identical with Procedure A but the silver ion concentration is 0.0025 M and contains only 5 drops of 1 M  $\text{Na}_3\text{NTA}$ . Samples processed by this procedure have less fog than those processed by procedure A.

## EXAMPLE 6

Titanium dioxide coated sheets are exposed for 3 seconds on a print box to line negative and held for 10 seconds. The sheets are then immersed for 10 seconds in 0.0005 M  $\text{AgNO}_3$  which is 0.001 M  $\text{Na}_3\text{NTA}$  and drained for 5 seconds. The sheets are then immersed for 15 seconds in the following solution:

|                      |        |
|----------------------|--------|
| 1M $\text{CuSO}_4$   | 20 ml. |
| 1M CuEDTA            | 20 ml. |
| developer (Ag)       | 5 ml.  |
| $\text{H}_2\text{O}$ | 55 ml. |

Developer (Ag) is a solution of p-methylaminophenol (2g./l.) and  $\text{Na}_2\text{SO}_3$  (7.5g./l.). After draining for 5 seconds, the sheets are immersed in TiEDTA developer (described in Example 1) for 5 seconds and washed for 5 seconds.

The images are of excellent density and high contrast.

## EXAMPLE 7

Titanium dioxide coated sheets are exposed for 3 seconds on a print box, held for 10 seconds, immersed for 10 seconds in 100 ml. of 0.0005 M  $\text{AgNO}_3$  which contains 2.5 ml. 1M  $\text{Na}_3\text{NTA}$  and drained for 5 seconds. The sheets are then immersed for 15 seconds in 0.3 M CuEDTA (prepared with  $\text{CuSO}_4$ ) and drained for 5 seconds and then developed in TiEDTA developer (described in Example 1) for 5 seconds and finally water washed. The prints obtained are of excellent density.

When this procedure is repeated omitting the  $\text{Na}_3\text{NTA}$  from the silver ion solution, the prints obtained are of lower density than those produced with  $\text{Na}_3\text{NTA}$  present in the silver ion solution.

## EXAMPLE 8

Samples of a titaniumdioxide-coated paper are exposed on a sensitometer (stepwedge) for  $10^{-3}$  seconds and developed according to the following procedures:

1. immerse in 0.005 M  $\text{AgNO}_3$  for 10 seconds and drain for 10 seconds.
2. develop in a solution of p-methylaminophenol (2g./l.) and  $\text{Na}_2\text{SO}_3$  (7.5g./l.).
3. fix in aqueous  $\text{Na}_2\text{S}_2\text{O}_3$  for 1 minute and wash for 5 minutes.

B. Same as procedure A but 5 ml. of 1 M  $\text{Na}_3\text{NTA}$  is added per 100 ml. of  $\text{AgNO}_3$  solution.

Using Procedure A, the stepwedges show 15 steps for each of two sample sheets and with procedure B, two samples show 19 and 21 steps respectively.

When ethylenethiourea is added to the developer solution the number of steps increase:

- The procedures A and B are used with sample sheets exposed for  $10^{-4}$  seconds with similar results, Procedure A sheets showing 4 steps, while Procedure B sheets show eight steps.
25. Procedures A and B are repeated with sheets exposed for  $10^{-4}$  seconds but the silver nitrate concentration is increased to 0.03 M. The procedure A sheets show 7 steps while Procedure B sheets show 9 steps.

## EXAMPLE 9

Titanium dioxide coated sheets are exposed on a print box for 3 seconds, held for 10 seconds and processed by the following sequence:

- a. immerse for 10 seconds in 0.002 M  $\text{AgNO}_3$  containing 4 ml. of 1 M.  $\text{Na}_3\text{NTA}$  per 100 ml. and drain for 10 seconds.
- b. develop for 30 seconds in solution of p-methylaminophenol (4g./l.) containing 6 ml. of 1 M  $\text{Na}_3\text{NTA}$  per 100 ml. and drain for 10 seconds.
- c. immerse in  $\text{Na}_2\text{S}_2\text{O}_3$  aqueous solution for 1 minute and water wash.

The print shows 19 steps.

When  $\text{Na}_3\text{NTA}$  is omitted from the silver nitrate solution and the developer, the print shows 13 steps.

## EXAMPLE 10

Titanium dioxide coated sheets are exposed on a sensitometer (stepwedge), held for 10 seconds and processed according to the following sequence:

- a. immerse for 10 seconds in 0.002 M  $\text{AgNO}_3$  containing 4 ml./100 ml. of 1 M  $\text{Na}_3\text{NTA}$  and drain for 10 seconds.
- b. immerse for 15 seconds in a solution composed of:

|                         |        |
|-------------------------|--------|
| 1M $\text{CuSO}_4$      | 20 ml. |
| 1M Na <sub>3</sub> EDTA | 20 ml. |

## 60. Solution of p-methylaminophenol

|                      |        |
|----------------------|--------|
| (8 g./l.)            | 50 ml. |
| $\text{H}_2\text{O}$ | 5 ml.  |

and drain for 10 seconds.

- c. develop for 10 seconds in TiEDTA developer (described in Example 1) and drain for 10 seconds.

With an exposure time of  $10^{-3}$  seconds, the sheet shows 19 steps, with optical densities ranging from 1.09 to 0.82 (11th step).

When the immersion times are altered to (a) 5 seconds (b) 10 seconds and (c) 5 seconds and the drain periods to 5 seconds each, the sheet shown 21 steps with the same optical densities as the first sample, but with lower background fog.

## EXAMPLE 11

The procedure of Example 10 is repeated using 0.001 M  $\text{AgNO}_3$  containing 2.5 ml. of 1 M  $\text{Na}_3\text{NTA}$  per 100 ml. of solution to obtain sheets showing 18 steps. When the immersion time is shortened as described in Example 10, the sheets show 19 steps with a slight increase in optical density.

## EXAMPLE 12

The procedure of Example 10 is repeated using the following solution in step b:

|                                                             |        |
|-------------------------------------------------------------|--------|
| 1 M. CuEDTA (prepared with Cupric nitrate)                  | 30 ml. |
| 1M $\text{CuSO}_4$ , developer(Ag) (described in Example 6) | 10 ml. |
| $\text{H}_2\text{O}$                                        | 45 ml. |

The sheets show 21 steps with higher optical densities (1.21 for step 21) and lower fog.

When 5 ml. of 1 M  $\text{Na}_3\text{NTA}$  is added to the copper solution, the optical densities of the steps increase.

## EXAMPLE 13

Titanium dioxide coated sheets are exposed on a sensitometer (stepwedge), held for 10 seconds, and processed according to the following sequence:

- immerse for 10 seconds in 0.001 M  $\text{Ag}_2\text{SO}_4$  containing 50 ml. 1M  $\text{Na}_3\text{NTA}$  per liter and drain 10 seconds.
- immerse for 10 seconds in a solution composed of:

|                                                              |        |
|--------------------------------------------------------------|--------|
| 1M CuEDTA (from cupric Nitrate)                              | 30 ml. |
| 1M $\text{CuSO}_4$ , Developer (Ag) (described in Example 6) | 10 ml. |
| $\text{H}_2\text{O}$                                         | 10 ml. |
|                                                              | 50 ml. |

and drain 10 seconds.

- develop for 5 seconds in TiEDTA developer (described in Example 1)

Samples exposed for  $10^{-3}$  seconds showed 18 steps,  $D_{Max}=1.11$  and fog=0.11.

Sheets exposed to continuous tone negatives for  $10^{-2}$  seconds are processed using this procedure to obtain excellent prints of good resolution.

## EXAMPLE 14

Titanium dioxide coated paper sheet are exposed on a print box to a line negative for 3 seconds and processed according to the following sequence:

- immerse for 10 seconds in 0.0001  $\text{AgNO}_3$  containing 2.5 ml. of 1 M  $\text{Na}_3\text{NTA}$  per 100 ml. of solution and drain for 10 seconds.
- immerse for 30 seconds in developer (Ag) (described in Example 6) and drain for 10 seconds.
- immerse for 30 seconds in 0.25 M  $\text{CuSO}_4$  and drain for 10 seconds.
- develop for 30 seconds in TiEDTA developer (Example 1) and water wash.

The prints obtained are of good density and contrast. When the silver nitrate concentration is increased to 0.0005 M, prints of better density are obtained.

## EXAMPLE 15

The procedure of Example 14 is repeated using the following sequence:

- immerse for 10 seconds in 0.0005 M  $\text{AgNO}_3$  which is also  $1.25 \times 10^{1/2}$  M  $\text{Na}_3\text{NTA}$  and drain for 10 seconds.
- immerse for 15 seconds in 0.2 M CuEDTA containing 2g./l. p-methylaminophenol and 7.5 g./l.  $\text{Na}_2\text{SO}_3$  and drain for 10 seconds.
- develop for 5 seconds in TiEDTA developer (Example 1).

The prints show a good, black image corresponding to the negative.

## EXAMPLE 16

- The procedure of Example 10 is repeated using a solution of 0.5 M stannous chloride which is also 3.5 M  $\text{NaCl}$  in lieu of the copper amplifying solution. As reducing agent for stannous, a solution of chromous chloride (0.5 M) containing 2g./l. of glue and 0.3g./l. cresol is used. The developing time is a 30 seconds immersion in the reducing agent.

The stepwedge shows 18 steps and  $D_{Max}=0.74$ .

## EXAMPLE 17

- The procedure of Example 10 is repeated excepting that the source of nitriloacetate ions ( $\text{Na}_3\text{NTA}$ ) is applied to the photosensitive medium prior to photoexposure by immersion for 30 seconds in a 1 M solution of trisodium nitrilotriacetate, with equivalent results.

## EXAMPLE 18

- The procedure of Example 1 is repeated with the photosensitive medium being sensitized with the solution of silver nitrilotriacetate complex ion prior to photoexposure. Comparable images of good density and contrast are obtained.

## EXAMPLE 19

- The procedure of Example 7 is repeated using the following treating steps:

- immerse (after 10 seconds photoexposure) for 10 seconds in  $10^{-3}$  M. silver nitrilotriacetate complex ion solution and drain for 10 seconds.
- immerse in a solution of p-methylaminophenol (2g./l.) and  $\text{Na}_2\text{SO}_3$  (7.5g./l.) for 30 seconds and drain 10 seconds.
- immerse for 30 seconds in 0.5 M  $\text{SnCl}_2$  which is also 3.0 M  $\text{NaCl}$  and contains 5 ml. conc. hydrochloric acid/liter and drain for 10 seconds.
- immerse in freshly prepared 0.25 M chromous chloride in 1 M sulfuric acid solution for 30 seconds and then water wash.

An image of comparable density and contrast is obtained.

In the foregoing examples, the photosensitive media are principally paper and plastic film coated with the photoconductor. Similar results are obtained with metal foil coated with titanium dioxide, such as aluminum sheets coated with titanium dioxide, e.g., as described in commonly assigned copending U.S. application Ser. No. 446,707 filed Apr. 8, 1965, now abandoned.

## EXAMPLE 20

- A subbed triacetate film is coated with gelatin layer containing trisodium nitrilotriacetate. The dried layer is then coated with  $\text{TiO}_2$  in gelatin and dried. The medium is then imagewise exposed to light, immersed for 10 seconds in 0.00119 silver nitrilotriacetic acid, developed in a solution of p-methylaminophenol (2g./l.) and  $\text{Na}_2\text{SO}_3$  (7.5g./l.) for 15 seconds and then amplified with 0.25 M  $\text{CuSO}_4$  and TiEDTA developer solution as in the previous examples.

## EXAMPLE 21

- An anodized aluminum plate is coated with an aqueous slurry of  $\text{TiO}_2$  and polyvinyl alcohol and the coating dried. The medium is imagewise exposed to light and immersed for 10 seconds in 0.001 M  $\text{AgNTA}$  followed by development in p-methylaminophenol and  $\text{Na}_2\text{SO}_3$  as in Example 21. The medium is then amplified using steps (c) and (d) of Example 15.

## EXAMPLE 22

- A subbed triacetate film is coated with solution of CuEDTA in a suitable binder and dried. The coated medium is then coated with a slurry of  $\text{TiO}_2$  and  $\text{AgNTA}$  complex in a suitable

binder and dried in the absence of air. The medium is then exposed imagewise to light, optionally developed in a solution of p-methylaminophenol (2 g./l.) and  $\text{Na}_2\text{SO}_3$  (7.5 g./l.) and then immersed in titanous nitrilotriacetate developer for 30 seconds as in the previous examples to obtain an image of good density.

In addition to amplifying photographic images as described in the foregoing examples, the present systems and processes are also useful in the production of printed circuits as described in commonly assigned copending U.S. applications Ser. Nos. 721,778, filed Apr. 16, 1968 and 717,502 filed Apr. 1, 1968.

In the foregoing disclosure and in the attached claims, reference to the various metal complexes by use of conventional names, e.g., titanous nitrilotriacetic acid, ferrous ethylenediaminetetraacetic acid, silver nitrilotriacetic acid and the like, is intended to denote the complex ion made up of the indicated metal ion and an ion corresponding to the indicated acid. As is obvious to anyone skilled in the art, the stoichiometry of the complexes is not necessarily a simple 1:1 ratio but may vary somewhat according to the relative concentrations of the respective ions in solution. Since these complexes are formed readily from relatively soluble sources of the respective ions in solution and the additional ions of these sources in the solution do not adversely affect the formation of the desired complex, nor are they appreciably reactive in the oxidation-reduction reactions involving the desired complex, there is no need to designate the additional ions when referring to the complex. Of course, the additional ions are those remaining in solution and not involved in the complex formation, e.g., alkali metal ions, such as sodium or potassium ions, or ammonium ion from the source of complexing acid, and the negative ion of the metal salt introduced, e.g., sulfate, nitrate, halide and the like. Thus, the designation of the complexes by such expressions as titanous nitrilotriacetic acid, ferrous ethylenediaminetetraacetic acid and the like is intended to embrace the complex ions in solution, irrespective of the source of the respective ions which made up the complex. As mentioned hereinabove and as anyone skilled in the art will appreciate, the source of the respective ions should not contain ions which would adversely affect formation of the desired complex ion or adversely affect the oxidation-reduction reaction necessary for image amplification. Preferably, the selection of such ion sources should not result in precipitate formation between the negative ion of the metal ion source and positive ion for the complexing acid ion source. Thus, the salt of the complexing acid is preferably an alkali metal or ammonium salt both of which form soluble salts with most negative ions. In other words, the sources of silver ion and nitrilotriacetate ion, respectively, as well as the solutions thereof used in the photographic-development process used herein should contain only ions which are photographically acceptable and the environment in which they are employed should be photographically acceptable.

The following data is provided to illustrate the existence of the new silver complex of this invention:

Potential measurements were made on a solution of  $\text{Ag}^+$  and  $\text{NTA}^{3-}$  to show that complex formation occurred between these two ions. Some preliminary potential measurements were made on solutions whose potentials could be estimated. The potential of a 0.005 M  $\text{AgNO}_3$  solution can be calculated from the Nernst equation to be

$$\begin{aligned} E &= E^\circ + (0.059/1) \log [\text{Ag}^+] \\ &= 0.799 + (0.059/1) \log 5.0 \times 10^{-3} \\ &= -0.663 \end{aligned}$$

If the potential of this solution is measured against a saturated calomel electrode with an Ag electrode, the  $E$  cell value should be  $0.663 - 0.244 = 0.419$  V. A measured  $E$  cell of 0.425 V. was obtained for 0.005 M  $\text{AgNO}_3$  at pH 5.9 versus the saturated calomel electrode.

The effect of  $\text{EDTA}^{4-}$  on the  $\text{Ag}^+$ ,  $\text{Ag}$  potential was determined in view of the fact that  $\text{EDTA}^{4-}$  is known to form a complex with  $\text{Ag}^+$ . The equilibrium constant for the reaction,



is  $10^{7.32}$ , as given in "Stability Constants of Metal-ion Complexes," L. G. Sillen and A. E. Martell, Special Publication No. 17, The Chemical Society, London. The effect of complexation on the  $\text{Ag}^+$ ,  $\text{Ag}$  potential can be estimated by substituting the  $\text{Ag}^+$  concentration obtained from the formation constant into the Nernst equation:

$$\frac{[\text{Ag EDTA}^{3-}]}{[\text{Ag}^+] [\text{EDTA}^{4-}]} = 10^{7.32} [\text{Ag}^+] = \frac{[\text{Ag EDTA}^{3-}]}{10^{7.32} [\text{EDTA}^{4-}]}$$

$$E = 0.799 + \frac{0.059}{1} \log \frac{[\text{Ag EDTA}^{3-}]}{10^{7.32} [\text{EDTA}^{4-}]}$$

$$= 0.799 - 0.059 \log 10^{7.32} + 0.059 \log \frac{[\text{Ag EDTA}^{3-}]}{[\text{EDTA}^{4-}]}$$

$$E = 0.799 - 0.432 \text{ etc.}$$

$$E = 0.367 + 0.059 \log \frac{[\text{Ag EDTA}^{3-}]}{[\text{EDTA}^{4-}]}$$

This 0.367 V. is the new half-cell potential,  $E^\circ$ , for the half-reaction,



at a unit concentration ratio of the variable species. As a result of this formulation, and since the  $\text{Ag EDTA}^{3-}$  concentration is in the new Nernst equation, the reduction of the  $\text{Ag EDTA}^{3-}$  complex itself is being considered. At a unit concentration ratio of  $[\text{Ag EDTA}^{3-}]/[\text{EDTA}^{4-}]$ , a calculated  $E$  cell of  $0.367 - 0.244 = 0.123$  V. is obtained versus the saturated calomel electrode. A 0.005 M  $\text{AgNO}_3$ -0.010 M  $\text{Na}_3\text{NTA}$  solution was prepared. The solution was clear, colorless and at pH 10.6. If complexation occurs to any appreciable extent in this solution, the concentration of the complex should be close to 0.005 M and the free  $\text{EDTA}^{4-}$  should also be near 0.005 M and thus the ratio of species should be close to unity. The  $E$  cell for this solution was 0.169 V. versus the saturated calomel electrode. This value does not disagree to any great extent with the calculated 0.123 V. It was also found that a 0.005 M  $\text{AgNO}_3$  solution cannot remain soluble above pH 9.0 without precipitating out as the oxide. These two observations confirm that a soluble  $\text{Ag EDTA}^{3-}$  complex exists in a somewhat alkaline solution.

A 0.005 M  $\text{AgNO}_3$ -0.010 M  $\text{Na}_3\text{NTA}$  solution was prepared. A clear, colorless solution of pH 10.6 was obtained. The  $E$  cell of this solution versus the saturated calomel electrode was 0.252 V. The value of the half-cell potential,  $E$ , versus the normal hydrogen electrode is  $0.252 + 0.244 = 0.496$  V. The reduction reaction for the complexed species is:



and the corresponding Nernst equation is:

$$E = E^\circ + 0.059 \log \frac{[\text{AgNTA}^{2-}]}{[\text{NTA}^{3-}]}$$

If it is assumed that the concentration ratio  $[\text{AgNTA}^{2-}]/[\text{NTA}^{3-}]$  is close to unity, then the measured  $E$  vs. the normal hydrogen electrode is equal approximately to  $E^\circ$ . This  $E^\circ$  is related to an analogous way to the formation constant of  $\text{AgNTA}^{2-}$  as the  $E^\circ$  for  $\text{Ag EDTA}^{3-}$ . Thus,

$$\begin{aligned} E &= E^\circ - 0.059 \log K, \text{ Ag EDTA}^{3-} \\ 0.496 &= 0.799 - 0.059 \log K \end{aligned}$$

$$\log K, \text{ AgNTA}^{2-} = -\frac{0.496 + 0.799}{0.059} = 5.14$$

and



This value of  $K, \text{ AgNTA}^{2-}$  should be taken only as an approximate value at best.

A solution was prepared which was 0.005 M in  $\text{AgNO}_3$  and 0.005 M in  $\text{Na}_3\text{NTA}$ . The pH of this clear solution was 9.9 and  $E$  cell vs. SCE was 0.328 V. A fairly concentrated  $\text{HNO}_3$  solution was added dropwise, and the following data were obtained:

|                |       |       |       |       |
|----------------|-------|-------|-------|-------|
| pH             | 9.9   | 9.1   | 7.3   | 4.0   |
| E cell vs. SCE | 0.328 | 0.350 | 0.403 | 0.424 |

This last value is the same as that for a 0.005 M  $\text{AgNO}_3$  without any complexing agents present. This indicates that the portion was displacing the complexed  $\text{Ag}^+$ . The foregoing results indicate that at alkaline pH's,  $\text{NTA}^{3-}$  forms a complex with  $\text{Ag}^+$  having a relatively small formation constant as compared to the formation constants of  $\text{NTA}^{3-}$  with other metal ions.

What is claimed is:

1. In the method of rendering visible a latent image of an imagewise-exposed medium comprising a radiation-activatable photoconductor by converting said latent image to a silver latent image and amplifying said silver latent image with a physical developer, the improvement comprising:

contacting said exposed medium with a sensitizing solution containing silver ions in the presence of nitrilotriacetate ions, said solution having a pH of above about 4.

2. An improvement of claim 1 wherein said sensitizing solution comprises an aqueous solution having a concentration of silver nitrilotriacetate complex of from about  $1 \times 10^{-5}$  to about

5  $2 \times 10^{-1}$  moles per liter.

3. An improvement of claim 1 wherein said physical developer contains silver ions and a photographic reducing agent for silver ions.

4. An improvement of claim 1 wherein said physical developer contains copper ions and a reducing agent for copper ions.

5. An improvement of claim 1 wherein said physical developer contains tin ions and a reducing agent for tin ions.

10 6. In the method of rendering visible a latent image of an imagewise-exposed medium comprising a radiation-activatable photoconductor with a developer composition, the improvement comprising:

15 contacting said exposed medium with a solution comprising a complex of silver nitrilotriacetate.

7. An improvement of claim 6 wherein the concentration of said silver nitrilotriacetate complex is from about  $1 \times 10^{-5}$  to about  $2 \times 10^{-1}$  moles per liter.

8. A photographic medium containing a radiation-activatable photoconductor of titanium dioxide on zinc oxide as the photosensitive component thereof and a source of nitrilotriacetate ions.

\* \* \* \* \*

25

30

35

40

45

50

55

60

65

70

75